

Nov. 21, 1933.

M. M. ADLER

1,936,221

PYROTECHNICAL DEVICE

Filed May 13, 1932



INVENTOR  
Milton M. Adler,  
BY  
George D. Richards  
ATTORNEY

## UNITED STATES PATENT OFFICE

1,936,221

## PYROTECHNICAL DEVICE

Milton M. Adler, Newark, N. J.

Application May 13, 1932. Serial No. 611,110

8 Claims. (Cl. 102—20)

This invention relates, generally, to pyrotechnical devices or fireworks; and the invention has reference, more particularly, to a novel pyrotechnical device that is set into action by igniting the same and which provides a stick or handle adapted to be held in the hand of the user during the operation of the device.

Pyrotechnical devices commonly known as "sparklers" have sticks or handles for holding the same during use, and which, when ignited, produce a multiplicity of streamers or rays of light which project radially outwardly in all directions from the device, thereby forming a disk shaped flame extending at right angles to the stick portion of the firework, and which flame moves slowly toward the handle as the firework is consumed.

The principal object of the present invention is to provide a novel pyrotechnical device which differs from the sparkler type of firework in that the device of the present invention, though providing a handle adapted to be held by the user, yet produces, when ignited, an entirely different pyrotechnical effect which consists in the production of a succession of multiple small gleaming projectiles which fly off rapidly in all directions from the device and thereafter explode, producing beautiful little lights at various points.

Another object of the present invention lies in the provision of a novel pyrotechnical device comprising a stick or other suitable support having a portion of its length covered with a cylindrical layer of a pyrotechnical composition having a multiplicity of metallic granules or particles 35 adhered to the outer surface thereof, which metallic granules, during the ignition of the firework, are caused to fly off rapidly in all directions from the underlying pyrotechnical composition and thereafter burst into flame, producing tiny 40 explosions which may be of various colors.

Still another object of the present invention is to provide a novel pyrotechnical device of the above character, wherein the burning of the cylindrical layer of pyrotechnical material is progressive from one end of the layer to the other 45 end thereof, the said burning consuming an appreciable period of time which may be on the order of a minute or two, and as such burning progresses, the metallic granules are continuously 50 driven off in all directions to thereafter burst into flames with explosive effect, thereby producing continuously, small multiple explosions for an appreciable time.

Other objects of this invention, not at this time, 55 more particularly enumerated, will be clearly understood from the following detailed description of the same.

The invention is clearly illustrated in the accompanying drawing, in which:

Fig. 1 is a perspective view illustrating the novel

pyrotechnical device of the present invention in operation.

Fig. 2 is a view elevation of the novel pyrotechnical device; and

Fig. 3 is an enlarged sectional view taken along line 3—3 of Fig. 2.

Similar characters of reference are employed in all of the above described views, to indicate corresponding parts.

Referring now to said drawing, wherein the preferred embodiment of the novel pyrotechnical device of the present invention is illustrated, the reference numeral 5 designates the pyrotechnical device as a whole. Pyrotechnical device 5 consists of a substantially rigid supporting member 75 or stick 6 which may be made of wood or other suitable material. One end portion of the stick 6 is provided with a coating or layer 7 of a pyrotechnical composition which is applied to the stick 6 while such composition is in a plastic or 80 pasty condition. This layer or coating of pyrotechnical composition may be applied to the stick 6 as by dipping the latter into a vessel containing the plastic pyrotechnical composition.

The pyrotechnical composition constituting the 85 coating 7 is of such a nature that the same will harden as it dries out, but before this layer has had an opportunity to dry, and while the same is still in a plastic condition, a quantity of metallic or metallic alloy granules or particles 8 are 90 sprayed upon the exterior surface of the coating 7. The particles 8 in falling upon the coating 7, embed themselves slightly in the plastic composition thereof, thereby becoming stuck thereto, and as the composition dries, these granules become 95 firmly adhered to the layer 7 of composition and are disposed in surrounding relation thereto, thereby forming the completed device. The portion of the stick 6 not covered by the coating 7 provides a handle, whereby the device may be 100 held in use.

A composition found highly proficient for use in forming the layer 7 of the pyrotechnical device of the present invention consists in the use of the ingredients listed below, which are mixed 105 together in the following proportions, by weight:

|                     | Parts |
|---------------------|-------|
| Barium nitrate      | 85    |
| Strontium carbonate | 60    |
| Kryolith            | 40    |
| Potassium chlorate  | 110   |
| Dextrine            | 225   |
| Shellac             | 30    |
|                     | 55    |

The presence of the barium nitrate and strontium carbonate ingredients in the composition causes the latter, in use, to burn with a whitish-yellow flame, which color of flame results from the combination of the characteristic burning colors of these ingredients. These ingredients 115

also serve as combustibles and combine with the oxygen given off by the potassium chlorate to thereby maintain the combustion. The kryolith ingredient (made by De Haem Co.) apparently 5 serves as a flux and aids in obtaining uniform burning while the shellac and dextrine ingredients serve as binders.

In preparing the composition, the several ingredients in the proportions given above are 10 thoroughly mixed together, and sufficient water is added thereto to form a thick paste or plastic material. The sticks 6 are dipped into this plastic material and then removed causing a layer 7 of the material to adhere to the sticks. While the 15 layer 7 is still plastic, the granules or particles 8 are sprayed thereon as by shaking sieves containing the granules 8 above the sticks 6 and while turning or rotating these sticks which are preferably held in horizontal positions during the 20 spraying operation, so as to thereby cover the entire surface of the layer 7 with these granules.

As the layer 7 of composition dries out it 25 hardens, thereby firmly uniting the granules 8 to the surface portion of this layer. The dried composition 7 is relatively hard and dense and is non-hygroscopic and keeps well under variations of climatic conditions. This composition 30 is not subject to spontaneous combustion and will remain properly operative for the purposes intended for an indefinite period.

The granules 8 are preferably composed of rapid 35 burning metallic alloys although pure metals such as magnesium or aluminum in some instances may be used. Alloys of magnesium and aluminum with metals of higher melting points are preferred to the pure metals, however, because such alloys, having higher melting points than these pure metals themselves, do not tend to melt too rapidly while in contact with the burning composition 40 7 but instead are caused by the generated gases to fly off in solid form and thereafter burn with explosive violence, as desired. Alloys of magnesium and copper or aluminum and copper have been found highly satisfactory for this purpose.

In use, the firework is held by the handle portion of stick or rod 6 and the composition 7 at the outer tip of the rod is ignited causing this composition to burn with an attractive colored 50 flame. As soon as the composition 7 commences to burn, the granules 8 in the proximity of the flame are caused to be driven off from the firework at relatively high speeds in all directions as especially shown in Fig. 1. These granules 55 glow somewhat as they move through the air, thereby creating the effect of a multiplicity of streamers moving rapidly away from the firework. After these granules have traveled to varying distances from the firework, they burst into 60 flame or explode, thereby producing beautiful little lights or whiffs of flame 9 of varying colors, depending upon the composition or compositions of the metallic alloys used in making the granules 8.

65 The burning of the layer of composition 7 progresses slowly down the stick 6 and as this burning continues, the glowing granules 8 are continuously driven off of the firework and thereafter burst into little flames producing a novel 70 pyrotechnical effect. This display continues until the entire layer 7 of the composition is con-

sumed which may take a minute or two or even longer, depending upon the length of this layer 7.

As many changes could be made in the above construction and many apparently widely different embodiments of this invention could be 80 made without departing from the scope thereof, as defined by the following claims, it is intended that all matter contained in the above description or shown in the accompanying drawing shall be interpreted as illustrative and not in a limiting 85 sense.

What is claimed is:

1. In a pyrotechnical device of the character described, a body comprising, a combustible material, a binder, potassium chlorate as an oxidizing 90 agent and kryolith.

2. In a pyrotechnical device of the character described, a body comprising, a combustible material, a binder, potassium chlorate as an oxidizing 95 agent, kryolith, and metallic granules adhered to the surface of said body.

3. In a pyrotechnical device of the character described, a body comprising, barium nitrate as a combustible material, shellac as a binder, potassium chlorate as an oxidizing agent and kryolith, 100 and metallic granules adhered to the surface of said body, said granules comprising a bimetallic alloy.

4. In a pyrotechnical device of the character described, a body comprising, barium nitrate and 105 strontium carbonate as combustible materials, shellac and dextrine as binders, potassium chlorate as an oxidizing agent and kryolith.

5. In a pyrotechnical device of the character described, a body comprising, barium nitrate and 110 strontium carbonate as combustible material, shellac and dextrine as binders, potassium chlorate as an oxidizing agent, kryolith, and a multiplicity of metallic granules substantially covering and adhered to the surface of said body. 115

6. In a pyrotechnical device of the character described, a supporting stick, a pyrotechnical composition adhered to said stick in the form of a layer, and metallic granules or particles adhered to the surface of said layer, said granules 120 or particles being alloys of a plurality of different metals having different melting points, one of said metals being magnesium and another being copper.

7. In a pyrotechnical device of the character described, a body comprising, a combustible material, a binder, potassium chlorate as an oxidizing 125 agent and kryolith, and metallic granules adhered to the surface of said body, said metallic granules comprising an alloy of magnesium and copper.

8. In a pyrotechnical device of the character described, a body having a multiplicity of metallic granules partially embedded in the outer surface thereof, said body comprising a mixture of 130 the herein named ingredients in approximate proportions by weight as follows:

|                     | Parts |
|---------------------|-------|
| Barium nitrate      | 85    |
| Strontium carbonate | 60    |
| Kryolith            | 40    |
| Potassium chlorate  | 140   |
| Dextrine            | 225   |
| Shellac             | 30    |
|                     | 55    |

MILTON M. ADLER.

145